

# UNITED STATES PATENT OFFICE.

JAMES R. ROSE, OF EDGEWORTH, PENNSYLVANIA, AND JOHN HARRIS, OF LAKEWOOD,  
OHIO, ASSIGNEES TO CARBO-OXYGEN COMPANY, OF PITTSBURGH, PENNSYLVANIA,  
A CORPORATION OF DELAWARE.

## GASEOUS FUEL.

1,404,236.

Specification of Letters Patent. Patented Jan. 24, 1922.

No Drawing.

Application filed December 26, 1919. Serial No. 347,463.

To all whom it may concern:

Be it known that we, (1) JAMES R. ROSE, (2) JOHN HARRIS, citizens of the United States, residing at (1) Edgeworth, (2) Lakewood, in the county of (1) Allegheny, (2) Cuyahoga, and State of (1) Pennsylvania, (2) Ohio, have invented a certain new and useful Improvement in Gaseous Fuel, of which the following is a full, clear, and 10 exact description.

This invention relates to gaseous fuel which is particularly useful for the purpose of producing a concentrated flame having a high flame temperature and capable of 15 doing extremely fine work in the cutting of metals. A flame of this character is requisite for use in blowpipes with carbographs and for the cutting of steel such as is used in die work and for the trimming of the 20 edges of armor plate as at present constituted.

We obtain a gas having the above desirable characteristics by mixing with hydrogen, as a combustible base, methane and by-product coke-oven gas in the proportions of 25 from 2½% to 12½% by volume each of such methane and by-product coke-oven gas to the hydrogen constituent. The by-product coke-oven gas and the methane have 30 nearly the same flame temperature as the hydrogen, and the temperature produced by the combustion of the combined or mixed gases is nearly 3200° C. The by-product coke oven gas is readily obtainable in steel mills and the methane is 35 the main constituent of natural gas. The gaseous mixture produces within the burning hydrogen a visible cone which enables the operator to adjust the proportions of the 40 gases and of the combustion-supporting oxygen as may be necessary, as well as to apply the flame in the most advantageous manner to the work. Both the volume of the flame and the heat units produced by the combustion 45 of the mixture are greater than are produced by the combustion of hydrogen alone; and, as pointed out, the gaseous mixture is particularly well adapted for the cutting of metal with a minimum of slagging and with an extremely narrow slot, which results in the fineness of cutting referred to hereinbefore.

Taking Koppers by-product coke oven gas

|                                                                     |         |
|---------------------------------------------------------------------|---------|
| as a type, the average analysis of the same                         | 55      |
| CO <sub>2</sub> -----                                               | 2.6     |
| Illuminants -----                                                   | 4.3     |
| Oxygen -----                                                        | 0.2     |
| CO -----                                                            | 6.3     |
| Hydrogen -----                                                      | 46.3 60 |
| CH <sub>4</sub> -----                                               | 35.0    |
| Nitrogen -----                                                      | 5.3     |
| B. T. U. -----                                                      | 630     |
| Cu. ft. of oxygen required for combustion of a cu. ft. of gas ----- | 1.09 65 |

According to Richards on Metallurgical Calculations, published in 1908, and with the by-product coke-oven gas of approximately the analysis above set forth, the flame temperature produced by the combustion of the above described gaseous mixture will be about 3200° C., and the variations in the percentages of the said gases will cause approximately the following variations in 75 the net B. T. U. per cu. ft. of mixture and in the cubic feet of oxygen required for the combustion of a cubic foot of such mixture:

No. 1 mixture 95% H. with 2½% each of methane and by-product coke-oven gas; net 80 B. T. U.'s 317; cu. ft. of oxygen .550.

No. 2 mixture 75% H. with 12½% each of methane and by-product coke-oven gas; net B. T. U.'s 411; cu. ft. of oxygen .750.

Having thus described our invention, 85 what we claim is:

1. A gas for cutting, welding and heating purposes consisting of a mixture of by-product coke gas and methane with hydrogen in the proportions of from 2½% to 12½% 90 by volume of each of by-product coke gas and methane to hydrogen.

2. A gas for cutting, welding and heating purposes consisting of a mixture of by-product coke-oven gas and methane with 95 hydrogen in proportions not substantially less than 5% by volume of such combined gases to the hydrogen and not materially more than 25% of such combined gases to the hydrogen, the by-product coke-oven gas 100 and methane being present in the proportions of at least 2½% each in such mixture.

In testimony whereof, we hereunto affix our signatures.

JAMES R. ROSE.  
JOHN HARRIS.